

## UNITED STATES PATENT OFFICE

GUSTAVE LECOMTE, OF ROUSSILLON, FRANCE, ASSIGNOR, BY MESNE ASSIGNMENTS, TO  
DU PONT RAYON COMPANY, OF NEW YORK, N. Y., A CORPORATION OF DELAWARE

## LUBRICATION OF TEXTILE FIBERS

No Drawing. Application filed April 27, 1928, Serial No. 273,439, and in France December 24, 1927.

This invention relates to the art of dressing textile threads or fibers and more particularly to the dressing or coating of cellulose acetate threads or fibers.

Textile threads or fibers of all sources have been treated for the purpose of imparting to them luster, softness and flexibility or to facilitate the finishing operations. Due to the physical and chemical properties of the various fibers, it is desirable that the dressing produce other results. For instance, cellulose acetate threads or fibers have a tendency to show electrification phenomenon, and it is desirable in the treatment of these materials to choose a substance or composition which will counteract or offset this effect as well as dress the fibers.

The methods of treatment and compositions employed heretofore made use of various oils, such as mineral oils, drying oils or animal and vegetable oils. These oils, though they possess satisfactory dressing characteristics, have disadvantages which render their use unsatisfactory. Mineral oils, such as paraffin oil, vaseline oil and the like, have the disadvantage of not being saponifiable. Also they are very difficult to remove. These are serious faults with regard to the subsequent treatments of the thread or fiber and especially in dyeing. Drying oils, such as linseed oil, dry and form resins which are also very difficult to remove by any ordinary treatment. Animal and vegetable oils, such as olive oil and neat's-foot oil, though capable of saponification, have the unfortunate property of becoming rancid and of impregnating the thread or fabric with an objectionable odor which is difficult or impossible to remove.

I have found that I can overcome the above set forth disadvantages and produce a dressed or coated thread or fiber by using dressing compositions including oxidizing semi-drying vegetable oils. It is, therefore, an object of this invention to dress or coat threads or fibers with a composition which will impart the desirable characteristics without becoming rancid or resinified.

It is a further object of this invention to dress or coat threads or fibers with a com-

position which is capable of being easily removed and which will not interfere with the subsequent operations of the thread.

A specific object of this invention is to dress or coat cellulose acetate threads or fibers so that not only will the finishing operation thereof be facilitated but the electrification phenomenon thereof will be counteracted or suppressed. 55

A further specific object of this invention is to dress cellulose acetate fibers with a composition including an oxidized semi-drying vegetable oil. 60

I have found that I can attain these objects by using as a composition comprising an oxidized semi-drying vegetable oil of the cottonseed oil or rapeseed oil type. These oils may be obtained by blowing the semi-drying oil. Under a proper regulation of the conditions of oxidation oils having definite constants can be uniformly prepared. 65

These oxidized oils are very satisfactory for dressing textile fibers. When applied to the fibers, they impart a good smoothness and excellent texture. Due to their high viscosity 75 the oils keep the filaments in a compact bundle. They also are capable of producing stable and concentrated soapy emulsions without the use of emulsifying agents.

Furthermore, these oils can readily and easily be removed from the fibers by mere treatment with water at a low temperature. On storage there is no change in the odor of the oil or in the texture of the fiber. These oils are not subject to rancidity or oxidation 85 and are rather stable. When these oils are applied to cellulose acetate fibers they not only facilitate subsequent operations, but they also counteract, suppress or offset the electrification phenomenon. 90

These oils may be applied to the fibers in any one of various ways. For example, the oils, per se, may be applied to the fibers. If desired, the oils may be emulsified in water and the aqueous emulsion applied to the fiber; or, the oils may be dissolved in some solvent, preferably volatile, and the solution applied to the fibers. The oil, emulsion, or solution thereof, is applied to the fibers in any suitable manner. If an emulsion of oil is used, the 100

impregnated or coated fabric is subsequently subjected to a drying to remove the water. In case a solution of oil in some volatile solvent is used, after application to the fibers, the solvent may be recovered by any well known means.

In order to more clearly explain this invention the following specific examples are set forth:

Example 1.—Oxidized rapeseed oil having an iodine number of 50-60 and a viscosity of 20-25 C. G. S. is emulsified in water with the aid of 2-6% of silk throwster's soap. A solution having a 20-25% concentration of the oil produces satisfactory results. It is obvious that other concentrations and emulsifying agents may be used.

Example 2.—Oxidized cottonseed oil is dissolved in heavy gasoline. The use of a solution containing 2-3% of oil has given satisfactory results. Concentrations and solvents other than those specifically set forth may be used. After application of this solution to the threads or fibers, the treated threads or fibers are dried and the solvent recovered.

Various materials may be added to the lubricating composition to produce special qualities. For example, if special qualities of texture, smoothness or cohesion are desired, small quantities of other lubricating or adhesive compounds or substances, such as olive oil, castor oil, sheep's wool grease and the like, may be added to the oil composition.

The invention is not intended to be limited to the precise and exact details as set forth above, since it is obvious that various modifications may be made without departing from the nature and scope of the invention.

I claim:

1. Textile fibers or threads coated with a composition comprising an oxidized semi-drying vegetable oil.
2. Textile fibers or threads coated with a composition comprising oxidized cottonseed oil.
3. Artificial textile fibers or threads coated with a composition comprising an oxidized semi-drying vegetable oil.
4. Cellulose acetate fibers or threads coated with a composition comprising an oxidized semi-drying vegetable oil.
5. Cellulose acetate fibers or threads coated with a composition comprising oxidized cottonseed oil.
6. Cellulose acetate fibers or threads coated with a composition comprising oxidized cottonseed oil and a small quantity of another lubricant.
7. Artificial textile fibers or threads coated with a composition comprising oxidized cottonseed oil.
8. Artificial textile fibers or threads formed of a cellulose derivative coated with

a composition comprising an oxidized semi-drying vegetable oil.

9. Artificial textile fibers or threads formed of a cellulose derivative coated with a composition comprising oxidized cottonseed oil.

10. Textile fibers or threads coated with a composition comprising oxidized rapeseed oil.

11. Artificial textile fibers or threads coated with a composition comprising oxidized rapeseed oil.

12. Artificial textile fibers or threads formed of a cellulose derivative coated with a composition comprising oxidized rapeseed oil.

13. Cellulose acetate fibers or threads coated with a composition comprising oxidized cottonseed oil.

In testimony whereof I have affixed my signature to this specification.

GUSTAVE LECOMTE.

90

95

100

105

110

115

120

125

130